

## UNITED STATES PATENT OFFICE.

DUNCAN MACRAE, OF EAST ORANGE, AND HENRY KNEELAND RICHARDSON, OF NEW-  
ARK, NEW JERSEY, ASSIGNORS TO WESTINGHOUSE LAMP COMPANY, A CORPORA-  
TION OF PENNSYLVANIA.

## GETTER AND THE APPLICATION THEREOF.

No Drawing.

Application filed June 8, 1922. Serial No. 566,847.

This invention relates to electrical devices comprising filaments adapted to be heated to incandescence and more particularly to substances to be applied to such filaments to increase the efficiency thereof.

An object of our invention is the provision of a method for causing getters or other beneficial substances to adhere to the filaments for electrical devices in a proper and efficient manner without using an organic binder.

Another object of our invention is the provision of an improved substance for increasing the efficiency of incandescent lamps and other electrical devices comprising incandescent filaments.

A further object of our invention is the provision of a fusible getter or the like containing an infusible or refractory admixture thereto, for the purpose of causing an even distribution of the getter on a filament and preventing the formation of fused beads of the getter substance on the filament.

A still further object of our invention is the preparation of a getter or the like comprising a refractory or infusible substance admixed with a fusible substance adapted to cause the refractory portion of the getter to adhere closely to an incandescent filament when the same is heated after the getter is applied thereto.

Other objects and advantages will be apparent as the description proceeds.

In the copending application Serial No. 470,672, MacRae, filed May 18, 1921, a getter and method of applying the same, and assigned to the Westinghouse Lamp Company, there is described a method of applying a getter consisting of cryolite which comprises fusing it to a filament for an incandescent lamp or the like. This method would be inapplicable to substances such as thoria, alumina, or other refractory materials which it might be desired to apply to a filament, because such substances cannot be fused conveniently in practice and, therefore, if used alone cannot be made to adhere to the filament.

Our invention obviates the above noted difficulty by providing a getter composed primarily of two constituents or classes of constituents. One constituent or class of constituents is refractory or infusible and may comprise thoria, cerium oxide, yttrium oxide, alumina, silica or a mixture of two or more of

the same. The other constituent or class of constituents of our improved getter is fusible and may comprise boric oxide, lithium fluoride, cryolite or a mixture thereof. The infusible constituent in the getter serves to cause an even distribution on the filament and prevent beading. The fusible constituent of the same serves to cause the getter to adhere strongly to the filament so that it will not be rubbed off during any of the usual manufacturing operations.

Our invention also contemplates a method of firmly affixing the getter to one or more of the parts of a lamp without the use of an organic binding material. It also aims to provide a method of introducing a getter into a lamp in a manner whereby the same is substantially free from adsorbed gases. By eliminating organic material and adsorbed gases, the present invention removes the necessity of providing a substance, such as phosphorus, to combine with such gases.

It has been found that the small amount of residual gas in a lamp after exhaustion may be efficiently disposed of by our getter which is also introduced to off-set the obscuring effect of volatilized filamentary material. Many kinds of material may be used in preparing a getter according to our invention, the requirements of our getter being that the materials used shall be beneficial to the lamp and that part of the getter shall be refractory or infusible and another part shall be more or less fusible. Although we have mentioned certain substances which we prefer to use in preparing our getter, it is to be understood that the same are merely illustrative and we are not restricted to their use.

The following description is of a preferred form of our getter and method of applying the same to a filament for an incandescent lamp, radio bulb, and the like. The getter material, which may consist of a mixture of thoria and cryolite in desired proportions, such, for example, as two parts of thoria and one part of cryolite, is preferably powdered and mixed with a liquid medium, such as water, to form a solution or suspension mixture, and is preferably applied to the filamentary material before the latter is mounted on the stem of a lamp. The filamentary material is passed through the getter suspension mixture, then through an electrically heated tube furnace and there the coating becomes heated

to a temperature high enough to dry, dehydrate and melt the fusible constituent or constituents, in this instance, cryolite. If the filament is composed of tungsten or other substance which readily oxidizes when heated, the coating should be fused thereon in an atmosphere of hydrogen or other non-oxidizing gas. This process causes the getter to become firmly affixed to the filamentary material and at the same time, expels adsorbed gases and reduces the surface area of the getter material to render it less adsorbent to gases.

It has been found that a fused coating of getter strengthens a filament, such as tungsten, so that the latter may be more readily handled without breaking. This additional strength is especially valuable in filaments of very small diameter, as such break very easily.

The filamentary material or wire when it has fused thereon a coating of getter, may be mounted on a spider for an incandescent lamp in the usual manner. After sealing the mount so formed in a bulb and the evacuation and tipping off of the same, the lamp may be lighted at its designed potential or normal voltage without the necessity of auxiliary apparatus to guard against short circuits therein, inasmuch as there is not present a sufficient quantity of gases to permit gaseous conduction on lamp voltages. When the lamp is lighted, the incandescent filament serves to vaporize a portion of the getter which, in such state, combines with the small amount of residual gas, chemically or physically, and, reaching the comparatively cool surfaces of the bulb, is condensed as an invisible deposit and there serves the purpose of adsorbing the ordinarily obscuring deposit of filamentary material which otherwise would cause blackening of the bulb.

The thoria, in the getter previously described in detail, may be replaced, in whole or in part, by cerium oxide, yttrium oxide, alumina or other similar refractory substances. The cryolite in the getter may be replaced, wholly or partly, by lithium fluoride, boric oxide, or similar fusible substances. Experience has shown, that a filament coated according to the present invention will resist the ordinary abrasion which may occur in manufacturing manipulations and retain such coating on the wire in substantially the full quantity applied. This is a distinct advantage, inasmuch as the amount of getter applied is a predetermined

quantity calculated for the greatest efficiency of the lamp.

The present invention is also applicable to the manufacture of vacuum or gas-filled tubes, which employ an electron-emitting element. Such elements of electron tubes may consist of an electrode coated with materials, such as oxides, which function as the primary electron-emitting element. It is desirable that the electron emission from such coated electrodes be constant in quantity, which requires that the coating be retained on the electrode without loss therefrom. The method disclosed in the present invention of firmly affixing such a refractory coating to an electrode will, therefore, be valuable in the manufacture of electron tubes.

While we have described what we now consider preferred means of practicing our invention, it is to be understood that many changes may be made therein within the spirit and scope of the appended claims.

What is claimed is:

1. The method of treating incandescent lamp filaments comprising applying a refractory getter thereto by means of an inorganic binder fused to the filament, introducing the filament into a bulb, exhausting the bulb, vaporizing the binder and thereafter vaporizing the refractory getter. 85
2. A filament for an incandescent lamp or the like evenly coated with a firmly adherent film comprising a refractory getter substance and an inorganic fusible substance the latter of which is fused onto the filament. 90
3. In an electric device comprising an evacuated sealed envelope, a filament having a firmly adherent coating consisting of a mixture of an infusible getter substance and a fusible substance the latter of which is fused onto the filament. 95
4. In an electric device a metallic filament comprising a firmly adherent coating of a mixture of thoria and cryolite adapted to be raised to incandescence by the initial application of normal voltage. 100
5. In an electric device comprising an evacuated sealed envelope, a metallic filament having fused thereon a uniform coating of a powdered mixture of thoria and cryolite. 110

In testimony whereof, we have hereunto subscribed our names this 7th day of June, 1922.

DUNCAN MacRAE.  
HENRY KNEELAND RICHARDSON.